

Patented Mar. 15, 1927.

1,620,940

# UNITED STATES PATENT OFFICE.

WARREN F. BLEECKER, OF BOULDER, COLORADO.

## PROCESS OF PRODUCING IMPERVIOUS MATERIAL.

No Drawing.

Application filed December 28, 1921. Serial No. 525,489.

This invention relates to the production of an impervious and chemical-resistant material and its principal object is to provide a material suitable for making conduits, vessels, containers and other articles used in laboratories and chemical plants or factories, which is impervious to liquids or gases and which is proof against the corrosive action of acids and other chemicals.

10 It is well known that artificial graphite while strictly chemical-proof, is by reason of its porosity not suitable for use in the production of apparatus employed to conduct or contain chemical liquids or gases, and it is another object of my invention to impregnate artificial graphite with a chemical-resistant substance so as to completely fill its pores and become a permanent and solid part thereof.

20 A further object of the invention is to render articles composed entirely or in part of artificial graphite, impervious by filling its pores or cells with a substance of high internal cohesion, and still other objects reside in providing a simple, economical and practical method of producing material and articles of the above described character.

With the above and other objects in view, my invention consists in impregnating artificial graphite with a preferably chemical-resistant substance of high internal cohesion, which by filling the voids and pores of the graphite, becomes a permanent and solid part thereof.

30 Particularly adapted for this purpose are bituminous or pyrogenous carbonaceous materials such as asphalt, tar and pitch which are substantially inert at ordinary temperatures and possess the degree of internal cohesion required to prevent the penetration of liquids or gases into the cells or voids they occupy.

The impregnation of the graphite with these substances, may be effected by placing it in a partial vacuum in a retort or other closed container which is heated to a temperature slightly above the melting point of the filler, and then introducing the latter in a melted condition into the evacuated space until the graphite is completely inundated.

40 The filler may, if so desired, be entered into the retort under pressure and by drawing its surplus off the graphite and cleaning the surface of the latter, the process of 50 impregnation is completed.

In order to render the impregnated

graphite resistant to all chemicals at any temperature, and impervious to all solutions and gases, it is baked by any suitable method in a kiln furnace or retort, care being taken 60 to exclude oxygen and thereby prevent oxidation of the material.

The baking step in the process of producing the material hardens and carbonizes the filler in the pores of the graphite and removes the volatile constituents thereof, and it may be repeated after re-impregnation of the object, as often as is necessary to completely fill the voids of the graphite with a hard and solid substance.

70 It will be evident that to expedite the hardening and carbonization of the hydrocarbonaceous filler after impregnation of the graphite, it is desirable to use one having a large percentage of non-volatile base 75 such as heavy asphalt, while to impregnate articles used only to carry or contain cold acids and the like, a light pitch such as that derived from the distillation of coal may be employed with satisfactory results.

80 Material made according to the present invention is of particular advantage in the manufacture of pipes and other conduits, valves, tools, dishes, concentrating pans, pumps and other apparatus in which a high 85 degree of resistance to chemical action together with complete imperviousness is a desideratum.

It will be understood that the artificial graphite may be impregnated and otherwise 90 treated, as hereinabove described, before or after the article is formed and that while a carbonaceous substance of the character referred to, is preferable, it is possible within the spirit of the invention to use a non-carbonaceous or inorganic, chemically inert material to fill the pores of the graphite so as to render it chemically resistant and impervious to liquids or gases.

95 The distinction which I make between 100 pitch and asphalt is that pitch is a coal tar product and asphalt is a natural product. The pitch has a lower melting point and impregnates easier and at a lower temperature and because of the presence of higher hydro-carbons is not so resistant to chemical action as asphalt. Asphalt carries a higher percentage of fixed carbon as well as a higher percentage of lower hydro-carbons.

105 What I claim and desire to secure by Letters Patent is:

1. The process of producing material of

the character described consisting in impregnating a body of artificial graphite with asphalt, baking the impregnated body and repeating the impregnating and baking 5 actions until the voids of the graphite are filled.

2. The process of rendering a body of artificial graphite impervious to liquids and gases consisting in immersing the body in a 10 liquefied chemical-resistant substance of high internal cohesion under a partial vacu-

um and completely filling and closing the voids of the artificial graphite.

3. The process of rendering a body of graphite impervious to liquids and gases 15 and consisting in immersing the body in liquefied asphalt under a partial vacuum and completely filling and closing the voids of the artificial graphite.

In testimony whereof I have affixed my signature.

WARREN F. BLEECKER.